

July 12, 1927.

K. B. LEWIS ET AL

1,635,945

MANUFACTURE OF WIRE DRAWING DIES

Filed March 14, 1924



Fig. 1.



Fig. 3.



Fig. 6.



Fig. 2.

Fig. 4.

Inventors:

Kenneth B. Lewis

Frank H. Ellsworth

By Owen W. Kennedy  
Attorney

## UNITED STATES PATENT OFFICE.

KENNETH B. LEWIS AND FRANK H. ELLSWORTH, OF WORCESTER, MASSACHUSETTS,  
ASSIGNORS TO MORGAN CONSTRUCTION COMPANY, OF WORCESTER, MASSACHUSETTS, A CORPORATION OF MASSACHUSETTS.

## MANUFACTURE OF WIRE-DRAWING DIES.

Application filed March 14, 1924. Serial No. 699,263.

Our invention relates to the manufacture of wire drawing dies and has for its object to provide an improved method of producing dies capable of accurately finishing more wire than dies heretofore employed for the same purpose. A further object of our invention is to provide an improved method, by the practice of which, large numbers of dies can be produced which will be absolutely uniform as regards the size and shape of the orifice through which the metal is drawn and all of which dies will have the same degree of hardness. A still further object is to provide an improved method capable of being carried on by comparatively unskilled operators with a consequent saving in manufacturing costs, as will herein-after appear.

In the manufacture of the wire drawing dies, the formation of the orifice, or hole, through which the metal is drawn, is of the utmost importance, and the accuracy of the die and the amount of metal which may be drawn therethrough is very largely determined by the manner of forming the hole. Therefore, in order that the nature and scope of our invention may be fully understood, there follows a brief discussion of the methods heretofore commonly employed in the manufacture of wire drawing dies.

In the production of dies composed of chilled cast iron, the holes are reamed to exact size by skilled operators, the reaming of the holes involving the actual removal of metal from the die. It is usually possible to draw only one bundle of wire through the hole of a cast iron die, after which the hole must be reamed out again to a larger size by a skilled operator, this procedure being followed after each draft until the hole becomes too large for the strength of the die and the die is scrapped.

In the production of steel dies to be used for drawing ordinary sizes of wire, a grade of steel is employed which will harden if heated and quenched. The usual practice when producing steel dies is to keep the metal in an annealed state, hardening the metal only in the immediate vicinity of the hole by cold working. When it is desired to reform a worn hole in a steel die, the worn-out hole is partially closed by hand hammering the metal around the same. This

hammering hardens the metal and at the same time crowds the metal into the hole so that, after hammering, the hole is smaller. The hammered hole is then enlarged to its original size by careful hand punching, which shapes and sizes the hole and further hardens the metal. The restoring of a hole to size requires considerable skill and experience on the part of the operator, for the hammering must neither be too heavy nor too light, and the blows must be evenly spaced around the hole and not too close to it. The tool with which the hole is punched to its final size is tapered, so that the size of the hole depends upon the depth to which the punch is driven. Therefore, great skill must be exercised by the operator when punching the hole, and the size of the hole must be tested after each blow on the punch. The operation of resetting holes in steel dies of this character is obviously slow and costly, the success of the operation depending largely on the skill and experience of the operator. It is usually possible to accurately draw but one bundle through a reset hole of a soft steel die.

In the drawing of large sizes of wire, which are to have only a slight reduction, steel dies have heretofore been employed to a limited extent which have been hardened by heating and quenching. In the production of such dies, a stream of water is passed through the orifice while the metal is red hot and in the resulting shrinkage of the metal, the opening becomes smaller than its original size. The opening is then restored to its original size by lapping, that is, by the use of a suitable rotating tool carrying an abrasive which removes the scale and brings the hole to true roundness. Hardened and lapped steel dies require much skill in their preparation, and both the dies and the holes must be so shaped as to secure uniform shrinkage.

From a consideration of the above, it is apparent that in all cases the working, or resizing, of the holes requires skilled operators, and that it is always difficult to obtain absolute uniformity in the sizes of holes owing to the fact that practically all the work is done by hand. Furthermore, an entire mill employing perhaps two hundred or three hundred men, may be thrown out of employ-

ment temporarily by the absence from work of two or three skilled die workers.

As previously pointed out, it is the object of our invention to provide an improved method of producing dies capable of accurately finishing more wire than either cast iron or soft steel dies as previously made, the practice of our invention permitting the production of large numbers of dies absolutely uniform as regards the size and shape of the opening and the degree of hardness of the metal. The production of dies by the practice of our invention is in no way dependent upon the manual skill of operators, the uniformity and quality of the product being assured by mechanical means, as will hereinafter more fully appear, reference being had to the accompanying drawings in which

20 Fig. 1 is a sectional view of a die at the time of carrying out the first step of our method.

Fig. 2 is a diagrammatic view illustrating means for carrying out the second step of our method.

Fig. 3 is a sectional view similar to Fig. 1, showing the appearance of the die after the performance of the second step.

Fig. 4 is a diagrammatic view illustrating means for carrying out the third step of our method.

Fig. 5 is a view of the punch used in Fig. 4.

Fig. 6 is a view similar to Fig. 1, illustrating the appearance of the die after the performance of the third step of our method.

Like reference characters refer to like parts in the different figures.

Referring to the drawings, Fig. 1 illustrates a usual form of die 1 preferably composed of a high grade of steel. The die is provided with a hole 2 originally formed, roughly, in any desired manner, at the time of making the die, and our invention has to do with the setting or resetting of this hole 2, preparatory to drawing wire therethrough. The hole 2 flares outwardly on one side of the die to guide the wire to the reduced cylindrical portion 2<sup>a</sup> of the hole which determines the size of the wire drawn therethrough in the direction of the arrow. In drawing wire through the cylindrical or reducing portion 2<sup>a</sup>, it has been found that the metal of the die is worn away, as indicated in dotted lines at a, a, in Fig. 1, thus forming an annular pocket surrounding the entrance to the reducing portion 2<sup>a</sup>. The formation of this pocket soon destroys the accuracy of the die which must then be reset. At this point it should be borne in mind that in the practice of our invention, it is immaterial whether the hole 2, shown in Fig. 1, is that of a new die which is to be set for the first time, or whether it is the worn hole 65 of an old die which is to be reset.

In carrying out our invention the die 1 is placed in a suitable heating furnace in which it is heated to a temperature well above its critical point. The furnace employed for heating the die is preferably of the type in which the degree of heating of the material therein may be controlled so that when a number of dies are successively placed in the furnace, all of them will be brought to substantially the same temperature.

The die having been heated to the desired degree, it is withdrawn from the furnace and immediately placed on the bed 3 of a hammering machine, diagrammatically illustrated in Fig. 2. The hammering machine is of the automatic type in which the hammering element 4 always operates in a uniform manner and is always adapted to strike an object placed on its bed 3 at the same rate and with the same force for a given setting of the machine. An automatic hammering machine of this type is fully shown and described in U. S. Patent No. 1,310,968, issued July 22, 1919, to Connor and Slinger, and it is not believed necessary to burden the present application with a detailed description thereof. Suffice to say that when the machine shown in Fig. 2 is set in operation, the hammering element 4 is adapted to strike the face 1<sup>a</sup> of the die 1 a series of blows distributed around the opening 2, the blows being delivered in a generally spiral path automatically determined by rotative movement of the bed 3 and simultaneous movement of the element 4 with respect to the axis of the die hole 2. For a given setting of the machine, the hammering of each die placed on the bed 3 is exactly the same and is carried on independently of the operator of the machine.

The above described hammering of the die 1 in its heated condition causes the metal therein to be somewhat condensed around the opening 2 so that the cylindrical portion 2<sup>a</sup> is, after hammering, slightly smaller than this portion was before being heated. The contraction of the opening 2 is shown on a somewhat exaggerated scale in Fig. 3, from which it is apparent that the pocket a shown in Fig. 1 has disappeared, and that an annular shoulder b has taken its place.

The hammered die 1 is then immediately placed, while still hot, on the bed 5 of a power punch, which is illustrated diagrammatically in Fig. 4. The punching tool 6 of this machine is the exact size and shape of the desired die opening and the machine is of such a type that upon release of its clutch, or other controlling device, the punching tool 6 is adapted to make one stroke in the die 1 to a predetermined depth. The tool 6 is shown in Fig. 5, from which it is apparent that the working stroke of the tool 6

in the heated die 1 shapes the hole 2 to the exact size and shape as shown in Fig. 6.

The punched die 1 is then moved from the punching machine, while still in a heated condition, and is dropped into an oil bath which serves to harden the metal by quenching.

The above described operations are adapted to be carried out in rapid succession, and each die that is handled in accordance with our method is treated in exactly the same manner. When a number of dies are being handled, they are all brought to the same temperature by the continuous heating furnace, after which the automatic hammering machine operates upon each of the dies in the same manner, the amount of hammering which each die undergoes not being susceptible of control by the operator. The dies are then all operated upon by the punching machine in exactly the same manner, the punch 6 always descending to the same point with relation to the bed 5, and with relation to the die face, so that the holes 2 produced in successive dies are identical in size and shape. By reason of the fact that each die is operated upon in exactly the same manner, the dies reach the oil at a uniform temperature and are consequently hardened to exactly the same degree.

We have found that dies produced by the practice of our invention being exactly uniform, as regards the size of the openings and degree of hardness, are also uniform in their behavior when used to draw wire, that is to say, a number of dies formed in accordance with our invention are adapted to produce wire of uniform size, and we have found that such dies will satisfactorily finish about six times as much wire as cast iron, or soft steel dies, used for the same purpose.

Furthermore, the production of dies in accordance with our invention can be carried on with much less labor and expense than has heretofore been necessary for setting of cast iron or steel dies. Obviously the heating, hammering, punching, and quenching of dies in accordance with our method can be carried on by comparatively unskilled operators, inasmuch as the hammering and punching machines are entirely automatic in their operation, while the degree of heating and cooling of the dies is determined entirely by the control of the heating furnace and the length of time it takes a die to be operated upon by the hammering and punching machines. The fact that the dies require no handling, other than the mere transfer from one machine to another, results in dies being set at a much faster rate by the practice of our invention than is possible when the setting is performed by the manual labor of skilled operators, as previously described.

While we are aware that the hammering and punching of dies has been heretofore carried on by hand, we believe that the automatic hammering of dies followed by hot power punching as a means of producing a finished hole, is entirely new. We have found in carrying out our invention that the quenching of the dies after hot punching results in the production of a finished hole which it is not necessary to lap out in order to polish the hole and free it from scale. This production of a finished hole by a single operation is doubtless due to the fact that the punch which enters and finishes the hole in the hot die leaves a film of oil which burns and protects the sides of the hole against oxidation until it is quenched.

We claim,

1. The improvement in the art of manufacturing wire drawing dies, which consists in heating dies to a uniform degree, automatically hammering the heated dies a uniform amount, power punching the heated dies in the same manner, and quenching the punched dies to obtain a uniform degree of hardness.

2. The improvement in the art of manufacturing wire drawing dies which consists in power punching a heated die by a single quick stroke to produce a finished hole therein, the punching being immediately followed by quenching to harden the die.

3. An improved method of making wire drawing dies, which consists in first heating a die a predetermined amount, then automatically hammering said die, then power punching said die by a single quick stroke to produce a finished hole, and finally in hardening said die by quenching.

4. An improved method of making wire drawing dies, which consists in first heating a die to a predetermined degree, then automatically hammering said die a predetermined amount, then power punching said die by a single quick stroke to produce a finished hole of a predetermined size, and then hardening said die by quenching.

5. An improved method of making wire drawing dies, which consists in first heating a die to a point above its critical temperature, then automatically hammering said die out of its original form, then power punching said die by a single quick stroke to produce a finished hole of predetermined size, and finally in hardening said die by quenching.

6. An improved method of making wire drawing dies, which consists in first heating a die to a predetermined temperature, then subjecting said die to the action of an automatic hammering machine which alters the shape of the die orifice a predetermined degree, then subjecting said die to a single quick stroke of a power punch with a tool of predetermined shape and size, which

penetrates said die to a predetermined depth, and finally in hardening said die by quenching.

7. An improved method of making wire drawing dies, which consists in heating a number of dies to the same degree, then hammering each of said dies a predetermined amount, then power punching each of

said dies by a single quick stroke to the same size and depth, and finally in uniformly <sup>10</sup> hardening each of said dies by quenching at the same temperature.

Dated this third day of March, 1924.

KENNETH B. LEWIS.

FRANK H. ELLSWORTH.